

## UNITED STATES PATENT OFFICE

WERNER FANSELAU, OF BERLIN-SIEMENSSTADT, GERMANY, ASSIGNOR TO SIEMENS & HALSKE AKTIENGESELLSCHAFT, OF SIEMENSSTADT, NEAR BERLIN, GERMANY, A CORPORATION OF GERMANY

ELECTROLYTIC PRODUCTION OF TIN FROM ALKALI STANNATE OR ALKALI STANNITE LYES

No Drawing. Application filed May 13, 1929, Serial No. 362,883, and in Germany May 16, 1928.

My invention relates to improvements in the production of tin, and more specifically to the electrolytic production of tin from alkali stannate or alkali stannite lyes.

5 The hitherto known and actually employed process for the electrolytic production of tin from alkali stannate or alkali stannite solutions in conjunction with soluble or insoluble anodes has the drawback that the tin deposited on the cathode is spongy and very porous, so that it is necessary to press it down continuously by rollers or the like in order to prevent it from dropping off the cathode. Only if very low current densities of the 10 order of about 50 amps. per square metre are employed is a fairly dense and smooth deposit possible, but even then such deposit can be obtained only in thin layers.

15 A more recent suggestion is to employ an electrolyte, which quantitatively contains only alkali stannate and besides this an addition of a colloid. This procedure leads to a satisfactory deposition of tin, but it is then impossible to work with soluble anodes, because the tin then dissolves in the two as well as in the four valence condition and oxidation of the lower valence tin to the higher valence tin is in this case practically impossible.

20 After extensive and thorough research I have ascertained that the spongy condition of the deposit of tin in the known process may be accounted for by the presence of an excess of free alkali. For example there is described in Foerster "The Electrochemistry of Watery Solutions", 3rd edition 1922, page 544, an electrolyte for detinning tinned sheet iron, which contains 10 p. c. total alkali (NaOH) besides 2 to 2.3 p. c. tin (Sn<sup>4+</sup>). This corresponds with a content of free NaOH of 25 8.65 to 8.45 p. c. If now according to my invention the content of the electrolyte in free alkali including the alkali liberated by hydrolysis is kept below 1.5 p. c., it is possible to obtain the tin in the form of thin, firmly 30 adhering coats of high lustre and great density (tinned sheet iron) as well as in thick, solid plates of dull silvery appearance without any spongy formations. My improved 35 process employs soluble anodes. Such an

electrolyte works absolutely satisfactorily at all concentrations of tin from 0.05 p. c. upwards to about 7 p. c. and at current densities from 50 amps. per square metre up to 1600 amps. per square metre. Preferably the content of free alkali is reduced as far as possible. When the concentration of free alkali rises considerably over 1.5 p. c. a dull, dirty-gray tin deposit which is inclined to become 40 spongy, is produced.

45 The process described above permits of a good solution of the problem for tin lyes of a concentration up to 7 p. c. If tin lyes of a higher concentration are used, it is found that it is generally impossible to avoid and increase in the content of free alkali beyond 50 1.5 p. c. due to the occurrence of electrolysis.

55 In a further development of the invention, especially for tin lyes of higher concentration, the deposition of spongy tin is avoided 50 by adjusting the ratio of the content of tin to the content of free alkali at 5:1. If, for instance, a tin lye is to be dealt with which contains 10 p. c. tin, the content of free alkali in this lye must be adjusted to 2 p. c. or 60 less.

65 As extensive experiments have shown, the adjustment of the ratio mentioned may be attained in all cases occurring in practice. I have also found that if the stated adjustment of the alkali content in relation to the content of tin is made, the deposition of spongy tin is also prevented in lyes of a concentration below 7 p. c. of tin, but it is possible 70 in such case to observe the relative concentrations described hereinbefore.

75 I claim:—

80 1. A process for the electro-deposition of tin from alkali stannate or alkali stannite lyes, which comprises adjusting prior to the 80 electrolysis the content of free alkali, including that liberated by hydrolysis, in dependence on the tin content of the lye, so that the ratio between the free alkali and the tin content is approximately 1:5, said process 85 employing soluble anodes, whereby said ratio is maintained during the electrolysis.

90 2. A process for the electro-deposition of tin from alkali stannate or alkali stannite lyes having a tin content below 7%, comprising 100

adjusting prior to the electrolysis the content of free alkali, including that liberated by hydrolysis, below 1.5%, said process employing soluble anodes, whereby said content of free alkali is maintained below 1.5% during electrolysis.

In testimony whereof I affix my signature.  
**WERNER FANSELAU.**

**10****15****20****25****30****35****40****45****50****55**